



US010240265B2

(12) **United States Patent**  
**McMaster**

(10) **Patent No.:** US 10,240,265 B2  
(45) **Date of Patent:** Mar. 26, 2019

(54) **METHOD FOR OPTIMIZING CONTACT RESISTANCE IN ELECTRICALLY CONDUCTIVE TEXTILES**

(71) Applicants: **Simon Adair McMaster**, Grantham (GB); **Footfalls and Heartbeats Limited**, Auckland (NZ)

(72) Inventor: **Simon Adair McMaster**, Grantham (GB)

(73) Assignee: **Footfalls and Heartbeats Limited**, Auckland (NZ)

(\*) Notice: Subject to any disclaimer, the term of this patent is extended or adjusted under 35 U.S.C. 154(b) by 522 days.

(21) Appl. No.: **14/765,943**

(22) PCT Filed: **Feb. 8, 2014**

(86) PCT No.: **PCT/IB2014/058866**

§ 371 (c)(1),  
(2) Date: **Aug. 5, 2015**

(87) PCT Pub. No.: **WO2014/122619**

PCT Pub. Date: **Aug. 14, 2014**

(65) **Prior Publication Data**

US 2015/0376821 A1 Dec. 31, 2015

**Related U.S. Application Data**

(60) Provisional application No. 61/762,346, filed on Feb. 8, 2013.

(51) **Int. Cl.**

**D04B 1/14** (2006.01)  
**D04B 1/10** (2006.01)  
**D04B 1/24** (2006.01)

(52) **U.S. Cl.**

CPC ..... **D04B 1/14** (2013.01); **D04B 1/10** (2013.01); **D04B 1/24** (2013.01); **D10B 2403/02431** (2013.01)

(58) **Field of Classification Search**

CPC . D04B 1/14; D04B 1/10; D04B 1/102; D04B 1/24

See application file for complete search history.

(56) **References Cited**

**U.S. PATENT DOCUMENTS**

4,087,991 A \* 5/1978 Robinson ..... D04B 1/106  
2/90

4,207,885 A 6/1980 Hampton et al.  
(Continued)

**FOREIGN PATENT DOCUMENTS**

DE 20209219 U1 8/2002  
DE 102008003124 A1 7/2009

(Continued)

**OTHER PUBLICATIONS**

International Search Report in related International Application No. PCT/IB2014/063929, dated Nov. 27, 2014.

*Primary Examiner* — Larry Worrell, Jr.

(74) *Attorney, Agent, or Firm* — Michele V. Frank; Venable LLP

(57) **ABSTRACT**

A method for optimizing contact resistance in electrically conductive yarns and textiles, and textiles having such optimized contact resistance, can include selecting a sensing activity for the textile; selecting a combination of variables from among yarn variables, stitch variables, and textile variables; and knitting an electrically conductive yarn in the textile in accordance with the selected combination of variables, wherein the knitted combination of variables provides an optimal contact resistance in the textile correlated with a desired electrical conductivity for the sensing activity. The knitted combination of variables can provide a predictable yarn contact area for the electrically conductive yarn correlated with the optimal contact resistance.

**13 Claims, 12 Drawing Sheets**



| (56)                  | References Cited                  |              |                   |         |                            |              |
|-----------------------|-----------------------------------|--------------|-------------------|---------|----------------------------|--------------|
| U.S. PATENT DOCUMENTS |                                   |              |                   |         |                            |              |
| 4,715,235 A           | 12/1987 Fukui et al.              |              | 8,948,839 B1 *    | 2/2015  | Longinotti-Buitoni .....   |              |
| 4,795,998 A           | 1/1989 Dunbar et al.              |              |                   |         | A61B 5/6804                |              |
| 6,080,690 A           | 6/2000 Lebby et al.               |              |                   |         | 29/825                     |              |
| 6,145,551 A *         | 11/2000 Jayaraman .....           | D03D 3/02    | 8,966,942 B2      | 3/2015  | Dias et al.                |              |
|                       |                                   | 139/387 R    | 9,032,762 B2 *    | 5/2015  | Begriche .....             | D04B 1/22    |
| 6,341,504 B1 *        | 1/2002 Istook .....               | A61B 5/0002  |                   |         |                            | 66/171       |
|                       |                                   | 2/69         | 9,186,092 B2      | 11/2015 | Mestrovic et al.           |              |
| 6,381,482 B1 *        | 4/2002 Jayaraman .....            | A61B 5/6805  | 9,282,893 B2 *    | 3/2016  | Longinotti-Buitoni .....   |              |
|                       |                                   | 600/388      |                   |         | A61B 5/6804                |              |
| 6,543,299 B2          | 4/2003 Taylor                     |              | 9,427,179 B2      | 8/2016  | Mestrovic et al.           |              |
| 6,941,775 B2 *        | 9/2005 Sharma .....               | A41D 13/1281 | 9,629,584 B2 *    | 4/2017  | Macia Barber ....          | A61B 5/04085 |
|                       |                                   | 2/902        | 9,808,196 B2 *    | 11/2017 | Macia Barber ....          | A61B 5/6804  |
| 6,970,731 B1          | 11/2005 Jayaraman et al.          |              | 9,817,440 B2 *    | 11/2017 | Longinotti-Buitoni .....   |              |
| 7,144,830 B2          | 12/2006 Hill et al.               |              |                   |         | G06F 1/163                 |              |
| 7,161,084 B2          | 1/2007 Sandbach                   |              |                   |         | 9,850,600 B2 *             | 12/2017      |
| 7,329,323 B2          | 2/2008 Dhawan et al.              |              | 2003/0224685 A1 * | 12/2003 | Gal .....                  | A61B 5/1135  |
| 7,365,031 B2          | 4/2008 Swallow et al.             |              |                   |         | Sharma .....               | A41D 13/1281 |
| 7,377,133 B2          | 5/2008 Sandbach et al.            |              |                   |         | 442/304                    |              |
| 7,544,627 B2          | 6/2009 Tao et al.                 |              | 2004/0009731 A1 * | 1/2004  | Rabinowicz .....           | A41D 13/1236 |
| 7,770,473 B2          | 8/2010 Von Lilienfeld-Toal et al. |              |                   |         |                            | 442/316      |
| 7,779,656 B2          | 8/2010 Dias et al.                |              | 2006/0258247 A1   | 11/2006 | Tao et al.                 |              |
| 8,116,898 B2 *        | 2/2012 Chung .....                | D04B 1/16    | 2007/0089800 A1   | 4/2007  | Sharma .....               |              |
|                       |                                   | 2/905        | 2008/0307899 A1   | 12/2008 | Von Lilienfeld-Toal et al. |              |
| 8,146,171 B2 *        | 4/2012 Chung .....                | D02G 3/36    | 2009/0013728 A1   | 1/2009  | Dias et al.                |              |
|                       |                                   | 2/167        | 2011/0015498 A1   | 1/2011  | Mestrovic et al.           |              |
| 8,191,433 B2          | 6/2012 Tao et al.                 |              | 2011/0030127 A1   | 2/2011  | Dias et al.                |              |
| 8,214,008 B2          | 7/2012 Hassonjee et al.           |              | 2013/0192071 A1   | 8/2013  | Esposito et al.            |              |
| 8,298,968 B2          | 10/2012 Swallow et al.            |              | 2016/0367191 A1   | 12/2016 | Esposito et al.            |              |
| 8,476,172 B2          | 7/2013 Christof                   |              |                   |         |                            |              |
| 8,669,195 B2          | 3/2014 Swallow et al.             |              | EP 1916323 A2     | 4/2008  |                            |              |
| 8,925,392 B2          | 1/2015 Esposito et al.            |              | EP 2809232 B1     | 12/2016 |                            |              |
| 8,945,328 B2 *        | 2/2015 Longinotti-Buitoni .....   | A61B 5/0002  | JP 2003-020538 A  | 1/2003  |                            |              |
|                       |                                   | 156/234      | WO 2004/100784 A2 | 11/2004 |                            |              |
|                       |                                   |              | WO 2004/100874 A2 | 11/2004 |                            |              |
|                       |                                   |              | WO 2009/093040 A1 | 7/2009  |                            |              |
|                       |                                   |              | WO 2012/101374 A1 | 8/2012  |                            |              |
|                       |                                   |              | WO 2014/080404 A1 | 5/2014  |                            |              |
|                       |                                   |              | WO 2014/122619 A1 | 8/2014  |                            |              |

\* cited by examiner

## FOREIGN PATENT DOCUMENTS



FIG. 1

| MER                      | SJ    | SP - A | SP - B | SP - C | SP - D |
|--------------------------|-------|--------|--------|--------|--------|
| Course - relaxed         | 0.129 | 0.022  | 0.017  | 0.011  | 0.020  |
| Course - tensioned       | 0.041 | 0.009  | 0.004  | 0.003  | 0.004  |
| Wale - relaxed           | 0.108 | 0.021  | 0.015  | 0.011  | 0.020  |
| Wale - tensioned         | 0.035 | 0.009  | 0.003  | 0.002  | 0.003  |
| Course - Dynamic Range % | 68    | 59     | 76     | 73     | 80     |

FIG. 2



FIG. 3A



FIG. 3B



FIG. 4



FIG. 5A



FIG. 5B



FIG. 5C



FIG. 6



FIG. 7



FIG. 8



FIG. 9



FIG. 10



FIG. 11



FIG. 12



FIG. 13



FIG. 14



FIG. 15



FIG. 16



FIG. 17



FIG. 18

| Temperature (°C) | Resistivity (KΩ) |             |
|------------------|------------------|-------------|
|                  | Polyester        | Merino Wool |
| 10               | 1.43             | 0.62        |
| 15               | 1.39             | 0.6         |
| 20               | 1.33             | 0.568       |
| 25               | 1.29             | 0.542       |
| 30               | 1.26             | 0.525       |
| 35               | 1.2              | 0.509       |
| 40               | 1.16             | 0.493       |

FIG. 19



FIG. 20

**METHOD FOR OPTIMIZING CONTACT  
RESISTANCE IN ELECTRICALLY  
CONDUCTIVE TEXTILES**

**FIELD OF INVENTION**

The present invention relates to a method for optimizing contact resistance in electrically conductive yarns and textiles, and textiles having such optimized contact resistance. Contact resistance can be optimized for particular desired uses of a yarn or textile product by adjusting physical, chemical, and/or mechanical variables in accordance with parameters predictable for such uses.

**BACKGROUND**

Constructing electrical circuits in textile materials presents a number of challenges. Conventional electrical circuits in textiles include conductive fibers knit or woven into a fabric, and capacitance or bioelectric sensors, transducers, or the like inserted into a textile structure. Such efforts have disadvantages, such as conductive fabrics that cannot be worn against a wearer's skin or must be limited to a small surface area. In garments having a sensor added to a fabric, design processes become complicated and manufacturing costs are increased.

An increasingly important field in textiles is that of "intelligent textiles" in which electrical signals representing physiological data are collected from garments and transmitted to remote locations, for example, for monitoring, assessment, and intervention by health care professionals. However, such textile devices are generally not truly "intelligent" textiles, as they comprise solid-state electronics placed in a textile shell and worn as apparel.

Previous efforts have been made to provide such "intelligent textiles." For example, one attempt includes a deformation-sensitive knitted or woven fabric structure of intertwined yarns having an electrical resistance that varies with degree of deformation. Another attempt to enhance electrical transmissions comprises a sensor array constructed from conductive threads in which the thread contacts are made with piezo-resistive junctions such that contact resistance changes with applied pressure. Another fabric includes a pressure-activated electrical sensor integrated into a knitted fabric such that fiber contact resistance can be related to compression force. Another knitted fabric that is designed to sense pressure and strain utilizes a single conductive yarn type, in which the applied pressure or strain causes different contact areas and resistances between adjacent loops of the yarn. In yet another example, a knitted electronic transducer utilizes a combination of conductive and non-conductive yarns such that extension in the course or wale direction causes loops in the transducer to separate or come together, varying the electrical resistance of the article. However, none of these efforts has addressed the optimal construction of a textile for suitably overcoming the challenges of contact resistance in such a device.

Thus, there is a need for a method for designing a textile structure to control the position and size of yarn contact areas for controlling electrical contact resistance and sensitivity of the structure to deformation. There is a need for such a method that utilizes a predictable stitch structure that improves control of contact resistance. There is a need for such a method that provides a means for varying a textile structure for specific applications. There is a need for such a method that allows use of a single conductive fiber type in a textile sensor. There is a need for such a method that allows

the textile structure to be utilized as a sensor for force, pressure, movement or temperature.

**SUMMARY OF THE INVENTION**

Embodiments of a method for optimizing contact resistance in electrically conductive yarns and textiles, and textiles having such optimized contact resistance, of the present invention can comprise selecting a sensing activity for the textile; selecting a combination of variables from the group consisting of yarn variables, stitch variables, and textile variables; and knitting an electrically conductive yarn in the textile in accordance with the selected combination of variables, wherein the knitted combination of variables provides an optimal contact resistance in the textile correlated with a desired electrical conductivity for the sensing activity. In some embodiments, the knitted combination of variables provides a predictable yarn contact area for the electrically conductive yarn correlated with the optimal contact resistance.

Other embodiments of a method for optimizing contact resistance in electrically conductive yarns and textiles, and textiles having such optimized contact resistance, can comprise selecting a combination of variables from the group consisting of yarn variables, stitch variables, and textile variables; and knitting an electrically conductive yarn having a yarn contact area in the textile in accordance with the selected combination of variables, wherein the knitted combination of variables provides a controllable amount of contact resistance in the textile. Some embodiments can further include selecting a sensing activity for the textile, and a controlled amount of contact resistance in the textile is correlated with a desired electrical conductivity for the sensing activity.

Some embodiments can further include selecting a measurement sensitivity for the sensing activity, and the knitted combination of variables can provide the optimal contact resistance in the textile correlated with a desired electrical conductivity for the measurement sensitivity. In various embodiments, the sensing activity can be selected from sensing tensile force, compressive force, movement, temperature, and physiological activity.

Some embodiments of a textile according to the present invention can comprise a sensing area comprising an electrically conductive yarn knitted in the textile and adapted for a sensing activity; and the sensing area comprising a combination of variables selected from the group consisting of yarn variables, stitch variables, and textile variables, wherein the combination of variables provides an optimal contact resistance in the textile correlated with a desired electrical conductivity for the sensing activity. In some embodiments, the combination of variables can comprise a predictable yarn contact area for the electrically conductive yarn correlated with the optimal contact resistance.

Some embodiments of a textile according to the present invention can comprise a sensing area comprising an electrically conductive yarn knitted in the textile; and the sensing area comprising a combination of variables selected from the group consisting of yarn variables, stitch variables, and textile variables, wherein the combination of variables provides a controllable amount of contact resistance in the textile. In such an embodiment, the sensing area can be adapted for a sensing activity, and a controlled amount of contact resistance in the textile can be correlated with a desired electrical conductivity for the sensing activity.

The combination of variables can be selected from yarn variables, including yarn type, yarn fabrication method, and

yarn count; stitch variables including stitch pattern, stitch length, and stitch percentage; and textile variables including electrical resistivity, fabric thickness, fabric weight, optical porosity, and percentage permanent stretch.

Features of a method for optimizing contact resistance in electrically conductive yarns and textiles and products having such optimized contact resistance of the present invention may be accomplished singularly, or in combination, in one or more of the embodiments of the present invention. As will be realized by those of skill in the art, many different embodiments of a method for optimizing contact resistance in electrically conductive yarns and textiles and products having such optimized contact resistance according to the present invention are possible. Additional uses, advantages, and features of the invention are set forth in the illustrative embodiments discussed in the detailed description herein and will become more apparent to those skilled in the art upon examination of the following.

#### BRIEF DESCRIPTION OF THE DRAWINGS

FIG. 1 is a diagrammatic view of two interconnected yarn units in a single jersey knit stitch pattern.

FIG. 2 is a table showing mean electrical resistivity (MER) values in a single jersey stitch pattern control and in four sample stitch patterns having different percentages of miss and tuck stitches. MER is shown for each stitch pattern having either relaxed or tensioned courses or relaxed or tensioned wales.

FIG. 3A is a diagrammatic view of a plain single jersey knit stitch pattern.

FIG. 3B is a diagrammatic view of a knit stitch pattern having single jersey stitches, miss stitches, and tuck stitches and showing yarn contact points in a tuck stitch in an embodiment of the invention.

FIG. 4 is a scanning electron microscope image of the yarn contact area for a single jersey, weft knitted fabric coated with polypyrrole (Ppy) conducting polymer in an embodiment of the invention.

FIG. 5A is a box plot showing variations in MER in the single jersey stitch pattern control and in the four stitch patterns having different percentages of miss and tuck stitches in FIG. 2. The range of MER is shown for each stitch pattern in a relaxed state in both the course direction and the wale direction.

FIG. 5B is a graph showing variations in fabric thickness relative to mean electrical resistivity in courses and in wales for the single jersey stitch pattern control and the four stitch patterns having different percentages of miss and tuck stitches in FIG. 2.

FIG. 5C is a graph showing variations in optical porosity relative to mean electrical resistivity in courses and in wales for the single jersey stitch pattern control and the four stitch patterns having different percentages of miss and tuck stitches in FIG. 2.

FIG. 6 is a graph showing variations in optical porosity relative to mean electrical resistivity in courses and in wales for a 50% plain single jersey stitch pattern.

FIG. 7 is perspective view of a test rig used to measure the effects of weight, or pressure, on stitch patterns having different percentages of miss and tuck stitches in the wale (vertical) direction and in the course (horizontal) direction.

FIG. 8 is a graph showing variations in electrical resistance caused by different amounts of weight in the course (horizontal) direction for swatches of the four stitch patterns having different percentages of miss and tuck stitches in FIG. 2.

FIG. 9 is a graph showing variations in electrical resistance caused by different amounts of weight in the wale (vertical) direction for swatches of the four stitch patterns having different percentages of miss and tuck stitches in FIG. 2.

FIG. 10 is a graph showing electrical resistance at a line directly below the ankle in the wale (vertical) direction for each of two sample stitch patterns having different percentages of miss and tuck stitches.

FIG. 11 is a graph showing electrical resistance at a line along the ball of the foot in the wale (vertical) direction for each of two sample stitch patterns having different percentages of miss and tuck stitches.

FIG. 12 is a diagrammatic view of the two interconnected yarn units in a single jersey knit stitch pattern shown in FIG. 1, showing yarn unit width, height, gap, and thickness.

FIG. 13 is an electron microscope photograph of a fabric sample comprising a multi-filament, twisted polyester yarn coated with silver knit in a plain single jersey stitch pattern in an un-deformed state.

FIG. 14 is an electron microscope photograph of a fabric sample comprising a stainless steel staple fiber spun yarn knit in a plain single jersey stitch pattern in an un-deformed state.

FIG. 15 is an electron microscope photograph of the fabric sample in FIG. 13 under a 22% strain in the wale direction, showing enhanced yarn contact compared to the un-deformed state.

FIG. 16 is an electron microscope photograph of the fabric sample in FIG. 15 under an 11% strain in the wale direction, showing similar yarn contact as in the un-deformed state.

FIG. 17 is an electron microscope photograph of the fabric sample in FIG. 15 under a 20% strain in the course direction, showing decreased yarn contact compared to the un-deformed state.

FIG. 18 is an electron microscope photograph of the fabric sample in FIG. 16 under a 12.5% strain in the course direction, showing slightly less yarn contact compared to the un-deformed state.

FIG. 19 is a table showing measured resistivities for each of a polyester and a merino wool sample at each of the seven tested temperatures.

FIG. 20 is a graph showing the resistivity measurements for each fabric sample in FIG. 19 plotted against the temperatures.

#### DETAILED DESCRIPTION

For the purposes of this description, unless otherwise indicated, all numbers expressing quantities, conditions, and so forth used in the description are to be understood as being modified in all instances by the term "about." Accordingly, unless indicated to the contrary, the numerical parameters set forth in the following description are approximations that can vary depending upon the desired properties sought to be obtained by the embodiments described herein. At the very least, and not as an attempt to limit the application of the doctrine of equivalents to the scope of the invention, each numerical parameter should at least be construed in light of the number of reported significant digits and by applying ordinary rounding techniques.

Notwithstanding that the numerical ranges and parameters setting forth the broad scope of the described embodiments are approximations, the numerical values set forth in the specific examples are reported as precisely as possible. Any numerical value, however, inherently contains certain

errors necessarily resulting from the standard deviation found in their respective testing measurements. Moreover, all ranges disclosed herein are to be understood to encompass any and all sub-ranges subsumed therein. For example, a stated range of "1 to 10" should be considered to include any and all sub-ranges between (and inclusive of) the minimum value of 1 and the maximum value of 10, that is, all sub-ranges beginning with a minimum value of 1 or more, and ending with a maximum value of 10 or less.

As used in this description, the singular forms "a," "an," and "the" include plural referents unless the context clearly dictates otherwise. Thus, for example, the term "a yarn" is intended to mean a single yarn or more than one yarn. For the purposes of this specification, terms such as "forward," "rearward," "front," "back," "right," "left," "upwardly," "downwardly," and the like are words of convenience and are not to be construed as limiting terms. Additionally, any reference referred to as being "incorporated herein" is to be understood as being incorporated in its entirety.

The following definitions are for purposes of the description herein:

"Contact Resistance": The equation

$$R_c = \frac{\rho}{2} \sqrt{\frac{\pi H}{F}}$$

is a representation of the Holm contact resistance equation, where  $R_c$  is contact resistance,  $\rho$  is material resistivity,  $H$  is material hardness, and  $F$  is the normal force. The equation

$$R_c = \frac{\rho}{2} \sqrt{\frac{\pi H}{nP}}$$

is another representation of the Holm equation, which is more relevant to textile based contact resistance.  $F$  is replaced by  $nP$ , where  $n$  is the number of contact points, and  $P$  is the contact pressure. Material hardness and electrical resistivity are constants that depend on the material properties of a textile. Contact resistance is therefore inversely proportional to the number of contact points and the contact pressure. That is, more contact points result in lower contact resistance. Therefore, as the number of contact points and/or contact pressure increases, contact resistance decreases. As used herein, contact resistance provides a measure of electrical conductivity in a yarn or textile. At the "micro" scale, surface roughness limits surface-to-surface contact. In addition, as pressure increases, the number of contact points increases, and eventually at the "nano" scale individual contact points "combine" into a larger contact area. "Integration as Summation" and the "Finite Element Method (FEM)" are techniques that can be used to determine the limits of these contacts points and therefore the contact area they produce.

"Course" is defined as a horizontal row of interlooped stitches running across the width of a knitted fabric.

"Force" is defined as any influence that causes an object to undergo a certain change, either concerning its movement, direction, or geometrical shape. In relation to a flexible textile network, force may be manifested as stretching, compression, or movement of the fabric structure.

"Miss stitch" is defined as a knitting stitch in which at least one needle holds the old loop and does not receive any

new yarn across one or more wales. A miss stitch connects two loops of the same course that are not in adjacent wales.

"Plain stitch" is defined as a knitting stitch in which a yarn loop is pulled to the technical back of a fabric. A plain stitch produces a series of wales or lengthwise ribs on the face of the fabric and courses, or cross-wise loops, on the back. A plain stitch can also be referred to as a "single-knit jersey stitch" or a "single jersey stitch."

"Tuck stitch" is defined as a knitting stitch in which a yarn is held in the hook of a needle and does not form a new loop.

"Wale" is defined as a vertical row of interlooped stitches formed by the action of one needle in successive courses along the length of a fabric.

Certain other definitions are provided elsewhere in this description.

The present invention can include embodiments of a method, or process, for optimizing contact resistance in electrically conductive yarns and textiles, and textiles, or textile products, having such optimized contact resistance. FIGS. 1-20 illustrate such embodiments. Contact resistance can be optimized for particular desired uses of a yarn or textile product by adjusting physical, chemical, and/or mechanical variables in accordance with parameters desired for such uses. An exemplary embodiment can comprise a method for designing and/or constructing a textile structure by controlling stitch pattern, percentage of different stitches within the stitch pattern, stitch density, yarn composition, yarn fabrication method, and/or yarn size.

Controlling such variables can control the number, location, and size (that is, quality) of yarn contact points (yarn contact area 52), and thus optimize the contact resistance and sensitivity of the textile structure for a particular type of measurement. The ability to control and adjust contact resistance for optimal sensor-specific electrical conductivity is due, at least in part, to the proportional relationships between stitch, yarn, and textile variables, or characteristics, and yarn contact area (52). For example, contact resistance can be controlled by inserting and removing various stitch types as a percentage of an overall knit structure so as to alter the size and shape of the yarn contact area (52). Such a method can take into account the three-dimensional complexity of a textile structure, including, for example, interactions of fibers within the yarn itself, and the relationship of controllable variables to electrical resistance characteristics during deformation of the textile structure.

In addition, selection and control of such stitch, yarn/fiber, and textile variables for providing optimal contact resistance for a particular use of a textile structure can be predictable, for example, a mathematically predictable selection of variables and correlated contact resistance.

In some embodiments, such a method for optimizing contact resistance can be applied to flexible electrically conductive yarns, textiles, and products. In some embodiments, knitted yarns can function as an electrically conductive sensor or network of sensors. Such a knit structure can be manufactured in such a way that it can be used to make a close-fitting and comfortable garment. The garment can be, for example, a compression garment, or a garment that acts in manner similar to a compression garment. In some embodiments, the textile structure can be formed within a conventional garment and utilized as a sensor. That is, the textile structure can have fully integrated knitted sensors, rather than electronic components inserted into fabrics as in conventional textiles. As a result, the textile structure can be customized so that sensors can be placed at various desired locations in the textile structure. Such sensors can be utilized

to measure force, pressure, strain, movement, temperature, physiological activity, and/or other variables.

In some embodiments, a method for optimizing contact resistance of the present invention can be applied to electrically conductive yarns, textiles, and textile products that are flexible. Control of contact resistance in a flexible network of electrically conductive yarn allows the textile structure itself to act as a sensing element. That is, "the textile is the sensor." In such an embodiment, no additional mechanical or solid-state electrical components are needed for the textile to measure desired variables. Some embodiments of a textile product having optimized contact resistance can be interchangeably described as "textile-as-sensor" or "textile-sensor."

Such a flexible textile-sensor in accordance with the present invention has a number of advantages. For example, one advantage is that as a result of the ability to control and optimize contact resistance, such a textile-sensor can effectively function in a variety of sensing applications. Another advantage of the ability to control and optimize contact resistance is that in a textile designed to perform a sensing function, conductivity can be enhanced for the type of signal being sensed so as to provide more accurate sensing and signal transmission. Another advantage of such a textile-sensor is that the shape of the sensor, or sensing area, can be controlled. The geometric shape of a sensor can affect how it functions. For example, in a textile-sensor utilized for sensing respiratory rate, a sensor, or sensing area, having the shape of a sine wave provides a clearer signal and uses less power than sensors having other shapes. In addition, the type and shape of sensor can affect how sensing activity interfaces with electronics for signal transmission and/or recording associated with the textile-sensor. Accordingly, differently shaped sensors in a textile-sensor can be advantageously utilized for different applications.

Another advantage of controlling electrical signals solely in a textile structure itself is that contact resistance can be optimized on macro scale ( $>2.5 \times 10^{-3} \text{ m}^2$ ) and on a nano scale. Another advantage of the ability to control and optimize contact resistance in the textile structure itself is that the textile-sensor can be customized to include any number of sensing areas. For example, such a textile-sensor can include a single, large sensing area or a plurality of smaller sensing areas. In certain embodiments, the textile-sensor capability can be combined with other fiber/yarn material characteristics to provide even further sensing functionality.

Another advantage of embodiments of such a textile-sensor is that the sensing structure can comprise a single layer of fabric. In contrast, conventional sensors, such as capacitive type sensors, can require multiple layers of fabric and fixed plates to function. Embodiments of such a textile-sensor can comprise a resistive sensor network that allows multiple types of sensing without the addition of fabric layers. As a result, some embodiments of such a textile-sensor can comprise a form-fitting, customizable garment that can be readily worn against the skin and thus allow a wide range of applications. For example, some embodiments of such a resistive textile-sensors placed against a wearer's skin can sense force changes in the wearer, such as respiration rate, mechanical joint movement, or strain during exercise. In certain embodiments, such resistive textile-sensors can perform physiological sensing, for example, sensing a heart rate signal, brain wave signal, or other muscle activity.

Some embodiments of a textile structure of the present invention provide advantages in comfort over conventional textile-based sensors. For example, conventional textile-

based sensors may be limited to woven and/or layered structures, which limit the number of materials suitable for use and/or prevent close skin contact without chafing. Existing sensors that require multiple layers of fabric and fixed plates to function also constrain comfort and wearability of a textile sensing device. Thus, another advantage of such a textile-sensor of the present invention is that without additional mechanical and/or electrical components or additional layers of fabric, a knitted textile-sensor can provide greater comfort and durability in a wearable product.

In embodiments of a method according to the present invention, optimizing contact resistance in electrically conductive yarns and textiles can comprise controlling and/or optimizing yarn variables, stitch variables, and/or textile variables so as to control and/or optimize yarn contact area (52).

Physical yarn variables, or yarn characteristics, that can affect contact resistance include, for example: (1) yarn type or composition; (2) yarn fabrication method; and (3) yarn count. Yarn type, or composition, influences yarn surface topography (surface roughness), and thus yarn contact area (52), in an electrically conductive yarn and/or textile. For purposes of this description, yarn type, or composition, includes characteristics such as whether a yarn is natural or synthetic, a staple fiber spun yarn, a filament yarn, single or multifilament, single or multi-ply, type and degree of twist, whether the yarn is textured, and/or other characteristics. Likewise, the method by which a yarn is fabricated, such as yarn spinning method, affects how the yarn influences yarn surface topography and yarn contact area (52).

Accordingly, yarn type, or composition, and yarn fabrication method affect contact resistance in a knitted fabric. Various electrically conductive fibers and yarns can be used to construct a textile structure having optimized contact resistance according to the present invention. For example, some embodiments of such a textile structure can be constructed using an electrically conductive silver yarn, or silver-coated yarn, an electrically conductive polyester-stainless steel yarn, or a combination of such yarns. Different types of yarn and different methods by which a yarn is made can affect yarn contact area (52) and contact resistance differently. Contact resistance-optimized textile structures comprising selected electrically conductive yarn types, compositions, and fabrication methods can be utilized in various applications to measure pressure, movement, and/or temperature.

Yarn count refers to the linear mass density of fibers and is defined as the mass in grams per 1000 meters. That is, yarn count is a measure of the size of a yarn. Yarn count correlates to yarn diameter and therefore yarn contact area (52). In particular, a yarn having a higher yarn count can provide a larger yarn contact area (52) and thus lower contact resistance.

Stitch variables, or characteristics, that can affect contact resistance include, for example: (1) stitch type, composition, or pattern; (2) stitch length; and (3) stitch percentage.

Stitch type, composition, or pattern influence yarn contact area (52), as shown in FIGS. 3 and 4. One common stitch type, shown in FIG. 3A, is a plain, single jersey stitch pattern 10. The single jersey stitch pattern 10 has interconnecting stitch loops 22, 24 that touch at single jersey contact points 42. The stitch type, composition, or pattern determines the configuration of the yarn in a textile, which influences the yarn contact area (52) and thus contact resistance.

Stitch length 20 is defined as a length of yarn which includes the needle loop 22 and half of the sinker loop 24 on either side of it. Generally, the longer the stitch length 20, the

more extensible and lighter the fabric, and the greater the potential number of yarn contact points (for example, 42, 44, 46, 48, 50). As shown in FIG. 3B, stitch length 20 and stitch composition have been altered from that shown in FIG. 3A, resulting in an increased number of contact points 42, 44, 46, 48, 50. Three stitches in a particular pattern provide an increased number of yarn contact points compared to the number of contact points provided by two stitches, which in turn provide an increased number of yarn contact points compared to the number of contact points provided by one stitch. Accordingly, stitch length 20 influences the yarn contact area 52 and thus contact resistance.

Stitch Percentage is defined as the percentage of stitch type in a stitch pattern. For example, stitch percentage can refer to the percentage of single jersey, miss, or tuck stitches 10, 34, 36, respectively, in a stitch pattern. Stitch percentage relates to fabric thickness. A stitch percentage that increases fabric thickness results in a larger yarn contact area (52), and therefore a corresponding decrease in contact resistance (and an increase in electrical conductivity). A stitch percentage variable, or metric, relates to a fabric/sensor at rest. When a force is applied, a fabric generally decreases in thickness.

Yarn contact area (52) has a direct influence on contact resistance of a textile structure. Contact resistance is associated with the conduction characteristic of the yarn contact surface area (52). The larger the yarn contact area (52) and the less the surface roughness of the yarn surface, the better the conductivity. An increase in yarn contact area (52) causes a proportional decrease in contact resistance. Yarn variables, stitch variables, and textile variables each influence yarn contact area (52), and thereby provide variables that can be used to control and/or optimize yarn contact area (52) and thus contact resistance and yarn conductivity.

Yarn contact area is illustrated in FIGS. 1, 3A, and 3B. FIG. 1 is a schematic representation of a single jersey stitch 10. In a single jersey knit fabric, a needle loop 22, or yarn unit, comprises a head 26 and two side legs 28 that form a noose 30. At the base of each leg 28 is a foot 32, which meshes through the head 26 of the loop 24 formed at the previous knitting cycle. The leg 28 of the needle loop 22 passes from one side (or face) to the other side/face of the sinker loop 24 across the leg 28 and head 26 of the sinker loop 24, and then loops around to pass back across the head 26 and opposite leg 28 of the sinker loop 24 to back to the original side/face of the sinker loop 24.

FIGS. 3A and 3B are schematic representations of stitch structures showing points of yarn contact. FIG. 3A is a schematic drawing of a single jersey stitch pattern. As shown in FIG. 3A, interconnecting stitch loops touch at single jersey contact points 42. In a single jersey stitch pattern, one stitch contacts an adjacent stitch essentially on only one side, or surface, of the adjacent stitch (or fabric) at a time. That is, in two interconnected stitch loops, the legs of a first stitch loop contact the feet of a second, adjacent stitch loop on one surface of the second stitch loop. On the opposite surface of the second stitch loop, the head of the first stitch loop contacts the legs of the second stitch loop. As a result, single jersey contact points are limited to relatively small crossover points of adjacent loops.

FIG. 3B is a schematic drawing of a single jersey stitch pattern having miss and tuck stitches. A single jersey stitch pattern having miss and tuck stitches includes single jersey contact points 42, as well as additional contact points at the miss and tuck stitches.

A tuck stitch contact point 44 occurs when a tuck stitch loop interconnects in a course with adjoining stitch types. As shown in FIG. 3B, in a tuck stitch, the leg of the stitch loop

passes around the head of an adjacent stitch loop. The leg of the tuck stitch loop contacts a first surface on one side of the head of an adjacent stitch loop. The leg of the tuck stitch loop then passes underneath to thereby contact a second surface of the head of the adjacent stitch loop at an angle substantially perpendicular to the first contact surface. Finally, the leg of the tuck stitch loop passes to the opposite side of the adjacent stitch loop so as to contact a third surface of the head of the adjacent stitch loop substantially perpendicular to the first contact surface and substantially parallel to the first contact surface.

It is understood that the contact(s) between the leg of the tuck stitch loop and the first, second, and third contact surfaces of the head of the adjacent stitch loop together form a continuous tuck stitch contact point (44) around the shape of the head of the adjacent stitch loop. As a result of this continuous contact configuration, the tuck stitch contact point 44 is approximately three times the size of the single jersey contact point 42. Due to the increased yarn contact area, the tuck stitch contact point 44 decreases contact resistance, as compared to the single jersey contact point 42.

A tuck loop contact point 46 occurs when the tuck loop of a tuck stitch presses upon the held loop of a tuck stitch. As shown in FIG. 3B, the head of the tuck loop contacts the head of the held loop along substantially the entire length of the heads of both the tuck loop and held loop. As a result, the yarn contact area (YCA) at the tuck loop contact point 46 is approximately one third the length of a tuck stitch loop length. Due to the increased yarn contact area, the tuck loop contact point 46 decreases contact resistance, as compared to the single jersey contact point 42. The tuck loop contact point 46 decreases yarn contact resistance when a textile incorporating tuck stitches is in a relaxed state or in a tensioned state.

A held loop contact point 48 is formed when the held loop of a tuck stitch is forced against an adjacent stitch loop. As shown in FIG. 3B, the head of the held loop of a tuck stitch contacts the foot of the adjacent stitch loop at the same point as the head of the tuck loop. The held loop contact point 48 has a similar size to the single jersey contact point 42, but provides a greater decrease in yarn contact resistance than the single jersey contact point 100 due to intrinsic stretch and recovery of a textile incorporating tuck stitches.

A tensioned tuck stitch contact point 50 is formed when a textile comprising tuck stitches is placed under tension. As shown in FIG. 3B (right hand portion), when the tuck stitch structure is placed under tension, the leg of the tuck stitch loop is forced into contact with the leg of an adjacent stitch loop. The yarn contact area of the tensioned tuck stitch contact point 50 is approximately one third the length of a stitch loop length. Due to the increased yarn contact area, the tensioned tuck stitch contact point 50 decreases contact resistance. The tensioned tuck stitch contact point 50 has a greater effect on yarn contact resistance when a textile incorporating such stitches is under tension.

As compared to the plain single jersey stitch pattern in FIG. 3A, the additional contact points 44, 46, 48, and 50 shown in the tuck stitch structures in FIG. 3B provide an increased number and quality of contact points. The quality of yarn contact points relates to factors such as the size of the surface area in contact between two or more portions of the yarn and the degree to which the contact points remain in contact as the textile, yarn, and stitches move during tensioning or deformation and relaxation. Accordingly, the tuck stitch contact points 44, 46, 48, and 50 provide increased yarn contact area and decreased contact resistance. Thus, embodiments of a method for optimizing contact resistance

## 11

in electrically conductive yarns and textiles can comprise knitting tuck stitches. Likewise, textiles having such optimized contact resistance can comprise tuck stitches. Optimizing, and thus controlling, contact resistance in electrically conductive yarns and textiles by varying the number and quality of tuck stitch contact points can be applied to various forms of knitted textiles in which such stitches are utilized.

FIG. 4 is a scanning electron microscope image of the yarn contact area 52 for a single jersey 10, weft knitted fabric coated with polypyrrole (PPy) conducting polymer. FIG. 4 shows the extent of yarn contact points 42 in this single jersey 10 fabric sample. When a conductive knitted fabric is subject to a load, the yarn contact area 52 increases due to suppression of any fabric surface roughness and compression of individual monofilaments into a large conductive fiber. Yarn contact area 52 increases in proportion to the total yarn circumference in contact and the total number of fibers involved.

As described herein, yarn type or composition and yarn fabrication method each influence yarn surface topography, or surface roughness, and thus the size and shape, or configuration, of a yarn contact area (52). Likewise, stitch type, composition, or pattern, stitch length, and stitch percentage each influence yarn contact area (52). Accordingly, these variables affect contact resistance between adjacent yarns in a knitted fabric. Different electrically conductive yarns have a different configuration of yarn contact points. For example, an electrically conductive polyester-stainless steel yarn has a first configuration (size and shape) of yarn contact points. An electrically conductive silver-coated yarn has a second configuration (size and shape) of yarn contact points different from the first yarn contact point configuration of the polyester-stainless steel yarn. However, embodiments of methods for optimizing contact resistance according to the present invention have the advantage of applying generally to the surface topography of all yarns. That is, the predictability of a particular selection of yarn and stitch variables to optimize contact resistance for certain applications can apply in general to any electrically conductive yarn.

In embodiments of a method according to the present invention, physical textile variables that can be controlled and/or measured in relation to optimizing contact resistance include: (1) mean electrical resistivity (MER); (2) fabric thickness; (3) fabric weight; (4) optical porosity (OP); and (5) percentage permanent stretch (PPS).

Electrical resistivity of electrically conductive fabrics is conventionally measured primarily using a four-point probe system, with the results produced in ohms/square. This method is primarily used to measure thin film or sheet resistance, and assumes that the thin film is two-dimensional, whereby resistance is calculated using the equation  $R=R_s(l/w)$ , where  $R_s$  is surface resistivity. Because textiles are three-dimensional, the depth dimension, although small relative to width and length, provides the basis for further contact points within a sensor structure. Therefore, for purposes herein, surface resistivity is measured in ohms and volume resistivity in ohms-cm ( $\Omega\text{-cm}$ ), or ohms cm ( $\Omega\text{-cm}$ ). Using a two-probe method, as described herein, allows for monitoring electrical signal output in both horizontal and vertical directions (measured in ohms-cm). Such a two-probe method can further allow monitoring of signal output through increments of  $360^\circ$  if probes are thusly attached on the sensor.

Mean Electrical Resistance (MER) ( $\text{k}\Omega\text{-cm}$ ) is defined as the measurement of the output that registers resistance in a

## 12

fabric. MER in a textile can range from about  $20\pm 1 \Omega\text{-cm}$  to about  $500\pm 15 \text{k}\Omega\text{-cm}$ . MER measured in the course direction is different from MER measured in the wale direction. In embodiments of the present invention, optimizing contact resistance optimizes mean electrical resistivity (MER). That is, as yarn contact area (52) increases, yarn contact resistance decreases, and MER decreases.

Fabric thickness (mm) impacts the ability to optimize conductivity in a fabric. As demonstrated in FIG. 5B, increased thickness improves conductivity. That is, as fabric thickness increases, yarn contact area (52) increases and contact resistance decreases. In the example in FIG. 5B, an increase in the contact area (52) between individual yarns is due to an increase in the percentage, or proportion, of miss (M) stitches 34 and tuck (T) stitches 36 with respect to the percentage, or proportion, of single jersey (SJ) stitches 10, and is demonstrated by increased textile thickness. For example, a combination of the SJ/M/T stitches with the miss stitch (34) 15% or less results in a thicker fabric than the SJ/M/T stitch combination with the tuck stitch (36) 15% or less. In some embodiments, fabric thickness can range from about  $0.5\pm 0.001 \text{ mm}$  and higher. A higher yarn count creates a larger fabric thickness and therefore larger yarn contact areas (52), and thus lower contact resistance and improved conductivity.

Fabric weight ( $\text{gm}/\text{m}^2$ ): As fabric thickness increases with respect to control of contact resistance so does the fabric weight. Therefore, as fabric thickness increases, fabric weight increases correspondingly, along with the same increase in yarn contact area (52) and decrease in contact resistance. An increase of miss and tuck stitches results in an increase in fabric weight due to the construction of miss stitches 34 and tuck stitches 36 in the knitting process. Miss stitches 34 and tuck stitches 36 cause an excess of yarn (in differing proportions) to build up in the textile structure compared to a single jersey 10 fabric. In some embodiments, fabric weight can range from  $100\pm 0.0001 \text{ gm.m}^2$  and higher. Embodiments having a larger yarn count (Tex/denier) and thus a larger fabric thickness also have a larger fabric weight, which, in turn, can decrease contact resistance and improve conductivity.

Optical porosity (OP) (% black pixels) is defined as a measure of the light that is transmitted through a fabric when tested using digitized images and analyzed using The University of Texas Health Science Center at San Antonio ImageTool software. Optical porosity provides a quantifiable measure of the cover factor of a fabric. "Fabric cover factor" is defined as the ratio of the area covered by the yarns to the whole area of the fabric. Optical porosity is measured as a ratio of black pixels to white pixels. A decrease in optical porosity corresponds to a decrease in contact resistance. Both miss and tuck stitches are formed when one or more stitches are removed from a plain jersey stitch 10 structure in either the weft (miss stitch 34) direction or warp (tuck stitch 36) direction. As with fabric weight, a change in the percentage, or relative proportion, of SJ/M/T stitches alters the amount of light that is able to pass through the fabric. A plain jersey stitch 10 provides a control structure with a fixed percentage of optical porosity. Thus, a change in the percentage of miss stitches 34 and/or tuck stitches 36 with respect to single jersey stitches 10 causes a change in the contact area (52) between yarns. An increase in tuck stitches 36 or a decrease in miss stitches 34 results in a decrease in optical porosity, depending on the relative percentage of miss stitches 34 and tuck stitches 36. Accordingly, an increase in yarn contact area (52) at rest, and a corresponding decrease in optical porosity, results in a

decrease in contact resistance. Therefore, a decrease in optical porosity is directly proportional to a decrease in contact resistance with respect to stitch patterns containing a combination of single jersey stitches **10**, miss stitches **34**, and tuck stitches **36**. Optical porosity can range from 1% black pixels and higher.

Percentage Permanent Stretch (PPS) is defined as a measure of the stretch and recovery of a fabric when subjected to a cyclical load. PPS increases or decreases depending on the percentage of miss stitches **34** and tuck stitches **36** within a particular stitch pattern. PPS relates to both the weft (course) direction **80** and warp (wale) direction **74**, and differs for each. The lower the PPS, the higher the optical porosity and therefore the lower the MER/contact resistance. PPS is directly proportional to the percentage of either SJ/M/T stitches present in the textile. Fewer miss stitches **34** in the courses reduce PPS in the weft/course direction **80**. Fewer tuck stitches **36** in the wales reduce PPS in the warp/wale direction **74**. Percentage Permanent Stretch can range from 25%-2%.

## EXPERIMENTS

The following experiments were conducted to test control of electrical conductivity in various such textile-sensor samples.

Experiments A, B, and C were conducted using the four textile samples in Table 1. Each sample comprises a different stitch pattern (SP). The yarn in each stitch pattern comprises 150 denier, **48** filament, 100% textured, multifilament, polyester coated in a polypyrrole (PPy) intrinsically conducting polymer. Each stitch pattern comprises 50% single jersey (SJ) stitches **10** and a different combination of miss (M) stitches **34** and tuck (T) stitches **36**. The percentage of miss stitches **34** and tuck stitches **36** are indicated for each stitch pattern in Table 1. In each of the experiments, a 100% single jersey stitch pattern **10** is used as a control for comparing the four sample stitch patterns (SP-A, SP-B, SP-C, and SP-D).

TABLE 1

| Textile Sample | Percentage of Stitches |          |          |
|----------------|------------------------|----------|----------|
|                | Single Jersey (SJ)     | Miss (M) | Tuck (T) |
| SP-A           | 50%                    | 5%       | 45%      |
| SP-B           | 50%                    | 10%      | 40%      |
| SP-C           | 50%                    | 45%      | 5%       |
| SP-D           | 50%                    | 40%      | 10%      |

### Experiment A

In Experiment A, mean electrical resistivity (MER), fabric thickness, and optical porosity in the four different sample stitch patterns were compared to those variables in a single jersey **10** fabric. The results of Experiment A, discussed with reference to FIGS. **2**, **5A**, **5B**, **5C**, and **6**, demonstrate how stitch patterns can be selected to affect these variables so as to optimize contact resistance in a textile.

The table in FIG. **2** shows mean electrical resistivity (MER) values in a single jersey (SJ) stitch pattern **10** control and in the four different sample stitch patterns. MER is shown for each stitch pattern having either relaxed or tensioned courses or relaxed or tensioned wales. Each of the four sample stitch patterns had significantly decreased MER in both the course (horizontal) direction **80** and wale (vertical) direction **74** in comparison to single jersey **10**, both in

relaxed states and in tensioned states. The discovery that each of the four sample stitch patterns had a significant effect on resting MER in both directions relative to single jersey allows selection of different stitch structures for different sensor types and/or sensing applications. In addition, each sample stitch pattern exhibited a decrease in MER between a relaxed state and a tensioned state, consistent with the effect of increasing yarn contact area (**52**) related to influence by tuck stitches **36** (such as the tuck loop contact point **46** and the tensioned tuck stitch contact point **50**) as the sample was tensioned.

In an embodiment of a method of the present invention, utilizing the resting MER and/or the dynamic range, or change, in MER from a relaxed state to a tensioned state for different stitch percentages allows control of sensitivity in a textile-sensor useful for a particular application. For example, the greater dynamic ranges (76%) in SP-B (10% miss/40% tuck) and (80%) in SP-D (40% miss/10% tuck) allow compressive force measurements over a greater force range in a compression garment or the like constructed from the fabric concerned. Such stitch patterns can be utilized to optimize contact resistance in a textile-sensor suitable, for example, for measuring compressive force in a sock. The smaller dynamic range (59%) in SP-A (5% miss/45% tuck) allows a more sensitive compressive force measurement for small force ranges. Thus, such a stitch pattern can be utilized to optimize contact resistance in a textile-sensor suitable, for example, for measuring force applied by a compressive bandage to a leg (for example, in the range about 10 mm Hg-60 mm Hg). In addition, the large percentage of miss, or float, stitches **34** (45%) in SP-C is associated with "waisting" in the textile-sensor. Waisting can be defined as the shape (for example, in extreme waisting, an hourglass shape) of a textile due to a higher percentage of miss stitches, which causes a decrease in course length as a result of less interlocking loops within each course. In a textile-sensor having a higher percentage of miss stitches, yarn contact area (**52**) increases and contact resistance decreases in a quantifiable manner.

FIG. **5A** shows variations in MER in the single jersey stitch pattern **10** control and in the four sample stitch patterns. A number of measurements of MER were taken for each stitch pattern in a relaxed state in both the course direction **80** and the wale direction **74**. The measurements were graphed in a box plot to show the ranges of variation. In FIG. **5A**, **Q0** represents the minimum measurement, **Q1** represents the bottom quartile of measurements, **Q2** represents the mean measurement, **Q3** represents the median measurement, and **Q4** represents the maximum measurement.

The range of MER variation in the single jersey stitch pattern **10** control and in the four sample stitch patterns varied depending on the stitch pattern. In particular, the range, or degree, of variation in MER in the single jersey **10** control was much greater than in the four sample stitch patterns. Accordingly, base calibration of resistivity in a single jersey stitch pattern **10** would be more difficult, resulting in a much less reliable textile-sensor structure than a textile-sensor structure having either of the four sample stitch patterns.

Optimizing contact resistance in an electrically conductive yarn or textile can comprise selecting a narrow range of MER variation. As shown in FIG. **5A**, SP-B (10% miss/40% tuck) and SP-C (45% miss/5% tuck) exhibited the most narrow ranges of MER variation. Thus, SP-B and SP-C comprise optimized contact resistance suitable for textile-sensor applications requiring greater measurement sensitiv-

## 15

ity. For example, SP-B and SP-C comprise contact resistance optimized for textile-sensor measurements of light weight pressures.

Fabric thickness is a measure of stitch density. FIG. 5B is a graph showing variations in fabric thickness relative to mean electrical resistivity in courses and in wales for the single jersey stitch pattern control and the four sample stitch patterns. As shown in FIG. 5B, as fabric thickness increases, MER decreases. In particular, the various combinations of miss stitches 34 and tuck stitches 36 in the four sample stitch patterns cause those stitch patterns to have a greater thickness than the single jersey stitch pattern 10. Accordingly, with the increased fabric thickness, the MER in each of the four sample stitch patterns is lower than in the single jersey stitch pattern 10 control, as measured in the course direction 80 and in the wale direction 74.

Likewise, optical porosity is a measure of stitch density. FIG. 5C is a graph showing variations in optical porosity relative to mean electrical resistivity in courses and in wales for the single jersey stitch pattern 10 control and the four sample stitch patterns. As optical porosity decreases (less light penetration), MER decreases, as shown in FIG. 5C. In particular, the various combinations of miss stitches 34 and tuck stitches 36 in the four sample stitch patterns cause those stitch patterns to have a lower optical porosity than the single jersey stitch pattern 10. Accordingly, with the decreased optical porosity, the MER in each of the four sample stitch patterns is lower than in the single jersey stitch pattern 10 control, as measured in the course direction 80 and in the wale direction 74.

FIG. 6 is a graph showing variations in optical porosity relative to mean electrical resistivity in courses and in wales for a 50% plain single jersey stitch pattern 10. As shown in FIG. 6, when increasing amounts of tuck stitches 36 and miss stitches 34 are added to a 50% single jersey stitch pattern 10, optical porosity decreases and electrical resistivity decreases.

Thus, fabric thickness and optical porosity, as measures of stitch density, were tested for correlations with MER. As shown in FIGS. 5B, 5C, and 6, it was discovered that both fabric thickness and optical porosity are strongly correlated with MER in a reliable manner across stitch patterns having different combinations of miss stitches 34 and tuck stitches 36. As a result, both fabric thickness and optical porosity can be utilized as simple measures in optimization of contact resistance in electrically conductive yarns and textiles. For example, a lower optical porosity in a fabric is associated with a greater contact area (52) between yarns (and lower MER) and therefore greater control of contact resistance. In other words, a more closed (more dense) stitch pattern having a lower optical porosity and greater yarn contact area (52) has greater measurement sensitivity in a textile-sensor than a more open (less dense) stitch pattern having a higher optical porosity and less yarn contact area (52). Thus, a more closed (more dense) stitch pattern having a lower optical porosity comprises optimized contact resistance suitable for textile-sensor applications requiring greater measurement sensitivity, such as for measurements of light compressive pressures or small tensile forces.

## Experiment B

In Experiment B, four fabric swatches, approximately 100 mm×100 mm in size, were knitted on a Shima Seiki WHOLEGARMENT™ 14 gg knitting machine. “gg” represents “gauge” of a knitting machine, and corresponds to the number of needles/inch. The yarn in each sample swatch

## 16

was a spun staple fiber yarn (80% PES/20% INOX®), commercially available as “S-Shield” from Schoeller. Each swatch was knitted using a different percentage combination of plain jersey stitches 10, tuck stitches 36, and miss stitches 34 (stitch patterns SP-A, SP-B, SP-C, and SP-D).

Individual sample swatches were then placed under weights in a test-rig 60, as shown in FIG. 7. The test rig 60 was constructed using 3 mm thick polymethyl methacrylate. Two stainless steel weights 62 were used, one weighing 150 gm, the other weighing 250 gm. The weights 62 were separated from the sample swatches by a non-conducting cardboard layer. One weight 62 remained in place on the sample being tested as a base weight to keep the area under pressure identical for each measurement. Each individual sample swatch was tested for electrical resistance measured with a Q-1559 multimeter (available from Dick Smith Electronics) using two standard multimeter probes 64. So as to compare data from both experiments, measures of electrical conductivity in Experiments B and C were taken as measurements of resistance, rather than resistivity, due to difficulty in obtaining accurate measurement of length under a person’s foot in Experiment C. Baseline resistance measurements were taken for each sample swatch without any weight 62 being applied. Ten resistance measurements were taken for each sample in a random manner under 150 gm of weight and under 400 gm of weight. The 400 gm of weight was applied by using the 150 gm weight 62 and the 250 gm weight 62 together. Measurements were taken with the multimeter probes 64 separated 28 mm and with an approximate pressure of 600 Pascal units (Pa) for the 150 gm of weight and an approximate pressure of 1000 Pa for the 400 gm of weight.

The results from Experiments B are represented graphically in FIGS. 8 and 9. FIG. 8 shows electrical resistance for baseline and for the 150 gm of weight and the 400 gm of weight in the course (horizontal) direction 80 for each sample swatch. FIG. 9 shows electrical resistance for baseline and for the 150 gm of weight and the 400 gm of weight in the wale (vertical) direction 74 for each sample swatch.

For the results shown in both FIGS. 8 and 9, the coefficient of determination, denoted  $R^2$ , was calculated.  $R^2$  indicates how well data points fit a statistical model, that is, a measure of how well observed outcomes are replicated by the model. In this instance, a high  $R^2$  value, or data fit, indicates a good linear relationship between the variables. With respect to these experiments, a high  $R^2$  value for a particular sample stitch pattern means that a textile-sensor comprising that stitch pattern can be utilized to measure weight/pressure in a reliable/repeatable manner.

The  $R^2$  values for stitch samples SP-A and SP-B are high for both the horizontal (course) direction 80 shown in FIG. 8 and the vertical (wale) direction 74, as shown in FIG. 9. Both SP-A (5% miss/45% tuck) and SP-B (10% miss/40% tuck) include a large proportion of tuck stitches 36, which serve to increase yarn contact area (52), and thus decrease—and thereby control—contact resistance, in both the vertical direction 74 and horizontal direction 80. Accordingly, stitch samples SP-A and SP-B demonstrate the best fit among samples tested for optimizing contact resistance in textile-sensors in accordance with the present invention.

In particular, the steeper gradient in the linear response by SP-B shown in FIG. 8 demonstrates a greater dynamic range in the course (horizontal) direction 80. Therefore, SP-B has a greater sensitivity to smaller amounts of weight in the course (horizontal) direction. Likewise, the steeper gradient in the linear response by SP-A shown in FIG. 9 demonstrates a greater dynamic range in the wale (vertical) direction 74.

Therefore, SP-A has a greater sensitivity to smaller amounts of weight in the wale (vertical) direction 74.

### Experiment C

In Experiment C, two fabric swatches, approximately 300 mm×100 mm in size, were knitted on a Shima Seiki WHOLEGARMENT™ 14 gg knitting machine. The yarn in each sample swatch was a spun staple fiber yarn (80% PES/20% INOX®), commercially available as “S-Shield” from Schoeller. Each swatch was knitted using a different percentage combination of plain jersey stitches 10, tuck stitches 36, and miss stitches 34 (stitch patterns SP-A and SP-B).

This experiment involved two human subjects. Subject 1 was female weighing 61 kg and subject 2 was male weighing 79 kg. Each subject stood, balanced only on her/his right foot, on the fabric swatches comprising the sample stitch patterns. Each subject wore a sock made from a non-conducting fiber. Each fabric swatch was tested for electrical resistance at two locations—at a line directly below the ankle and at a point approximating the ball of the foot). Resistance was measured on a Q-1559 multimeter (available from Dick Smith Electronics) using two standard multimeter probes 64. Ten resistance measurements were taken for each sample in a random manner at the two locations for each subject. A probe measuring separation of 70 mm was used for the ankle measurement, and a 100 mm separation was used for the ball of the foot measurement.

The results from Experiments C are represented graphically in FIGS. 10 and 11. FIG. 10 shows electrical resistance at a line directly below the ankle in the wale (vertical) direction 74 for each sample swatch. FIG. 11 shows electrical resistance at a line along the ball of the foot in the wale (vertical) direction 80 for each sample swatch.

A logarithmic regression, rather than linear regression, was used for the human-based results in Experiment C due to the large difference in mass applied to the sample fabric swatches as compared to that applied to the sample fabric swatches in Experiment B. Based on the  $R^2$  values for resistance measured at both the ankle shown in FIG. 10 and at the ball of the foot shown in FIG. 11, stitch sample SP-B demonstrates the best fit for use in certain embodiments of the textile-sensor in accordance with the present invention. In particular, the more shallow gradient in the logarithmic response by SP-B shown in FIGS. 10 and 11 demonstrates a greater response to larger amounts of weight. Therefore, stitch pattern SP-B provides a suitable textile-sensor for measuring pressure exerted by the human form. Considering the results of both Experiments B and C, it was found that stitch patterns SP-A and SP-B each provide optimized control of contact resistance useful in textile-sensors for measuring weight in different sized objects.

The findings of Experiments A, B, and C together demonstrate that making selections related to variables such as stitch pattern, stitch percentages, electrical resistivity, optical porosity, and fabric thickness can optimize contact resistance in electrically conductive yarns and textiles. Such a method can thus be utilized to reliably predict and control electrical conductivity capabilities in a textile structure and to design textile-sensors useful in a variety of applications. For example, a stitch pattern such as SP-B (10% miss/40% tuck) having: (1) a relatively large dynamic range in MER from a relaxed state to a tensioned state allows compressive force measurements over a greater force range; (2) a narrow range of MER variation allows textile-sensor applications requiring greater measurement sensitivity; and (3) a rela-

tively large dynamic range in MER in the course direction allows measurements in which a greater sensitivity to smaller amounts of weight in the horizontal direction are desired. Thus, a method of selecting stitch pattern, stitch percentage, and other physical stitch, yarn, and/or textile variables provides control of electrical conductivity in textiles such that predictable ranges and/or sensitivities of sensors can be constructed for particular uses.

10

### Experiment D

Experiment D was conducted to determine the effects of fabric deformation on the shape of yarn contact areas (52). In Experiment D, two fabric samples were tested. Sample A 15 comprises a multi-filament, twisted polyester yarn coated with silver knit in a plain, single jersey stitch pattern. FIG. 13 is an electron microscope photograph of Sample A in an un-deformed state. Sample B comprises a spun staple fiber yarn (80% PES/20% INOX®) in a plain, single jersey stitch 20 pattern 10. FIG. 14 is an electron microscope photograph of Sample B in an un-deformed state. In testing, measurements of multiple yarn units were taken, and descriptions of geometric parameters refer to average measurements in a sample.

25 The two fabric samples were first compared in an un-deformed state with respect to four geometric parameters of a yarn unit—width, height, gap, and thickness, as shown in FIG. 12. In a single jersey knit 10 fabric, the needle loop 22, or yarn unit, comprises the head 26 and two side legs 28 that 30 form the noose 30. At the base of each leg 28 is a foot 32, which meshes through the head 26 of the loop 24 formed at the previous knitting cycle. The leg 28 of the needle loop 22 passes from one side (or face) to the other side/face of the sinker loop 24 across the leg 28 and head 26 of the sinker 35 loop 24, and then loops around to pass back across the head 26 and opposite leg 28 of the sinker loop 24 to back to the original side/face of the sinker loop 24.

40 Yarn unit width (W) is defined as the distance between two feet 32 of a single loop 22 or 24. Yarn unit height (H) is defined as the distance between the head 26 and the foot 32 of a single loop 22 or 24. Yarn unit gap (G) is defined as the distance between the head 26 of one loop 22 and the head 26 of the adjacent loop 24 in the same wale. Yarn thickness (T) is defined as the diameter of a yarn. Sample A has a more 45 open knit structure, that is, a larger yarn unit width (W) and height (H) than Sample B. The yarn unit gap (G) is similar in the two samples. Sample B is thicker than Sample A.

The two samples were then compared in deformed states by stretching the samples first in the wale direction 74 (along the x-axis) and then in the course direction 80 (along the y-axis). “Stretching strain,” or the degree of stretching, is 50 defined as the ratio of yarn unit (loop) 22, 24 elongation to initial height. Sample A was tested under a similar strain as Sample B, as well as under a higher strain. The two samples 55 were compared in each state of deformation with respect to the four geometric parameters.

When the samples were stretched in the wale direction 74 (along the x-axis), the heads 26 of yarn loops 22 or 24 in one course were pulled tighter about the legs 28 and feet 32 of loops 22 or 24 in the adjacent course. As a result, the yarn 60 unit width (W) decreased significantly. During walewise stretching, yarn unit height (H) did not change significantly, but yarn unit gap (G) increases substantially. Yarn thickness (T) remained relatively unchanged.

65 For Sample A, under a walewise strain of 11%, yarn unit width (W) decreased about 19%, and the yarn unit gap (G) increased by about 16%, from comparative dimensions in

the un-deformed state. Under an 11% strain, the yarns contact at a few points. Under a walewise strain of 22%, yarn unit width (W) decreased about 39%, and the yarn unit gap (G) increased by about 26%, from the comparative dimensions in the un-deformed state. The photograph in FIG. 15 shows Sample A under a 22% strain **72** in the wale direction **74**. Under the 22% strain **72**, the yarns contact at every stitch. Thus, under loading in the wale direction **74**, a decreasing yarn unit width (W) and an increasing yarn unit gap (G) correlate with increasing yarn contact.

Therefore, under load in the wale (vertical) direction **74**, a decrease in yarn unit width (W) results in a less optically porous textile. As light penetration decreases and optical porosity increases, MER decreases. Accordingly, optical porosity can be used as an index of sensitivity to compressive or tensile force under load in the wale (vertical) direction **74** in an embodiment of a method for controlling contact resistance in a textile-sensor. Applying these results, a more closed (more dense) stitch pattern having a higher optical porosity comprises optimized contact resistance suitable for textile-sensor applications requiring greater measurement sensitivity, such as for measurements of light compressive pressures or small tensile forces. Therefore, a textile-sensor having a small yarn unit width (W) and corresponding lower optical porosity can be knit to increase contact resistance for such an application.

For Sample B, under a walewise strain of 11% (**76**), yarn unit width (W) decreased by about 1%, yarn unit height (H) increased by about 3%, and yarn unit gap (G) increased by about 3%, from comparative dimensions in the un-deformed state. The photograph in FIG. 16 shows Sample B under an 11% strain **76** in the wale direction **74**, showing similar yarn contact as in the un-deformed state. Sample B is significantly more compact than Sample A. That is, Sample B has a greater yarn unit thickness (T), and a smaller yarn unit width (W), yarn unit height (H), and yarn unit gap (G) than Sample A. As a result, Sample B has substantial yarn contact within a stitch even before deformation, or loading. As a result, the variation in geometric parameters for Sample B during loading in the walewise direction **74** is not as significant as for Sample A.

When the samples were stretched in the course direction **80** (along the y-axis), the legs **28** of the yarn loops **22, 24** were pulled apart from one another, such that the yarn unit width (W) increased. In addition, the yarn unit height (H) and the yarn unit gap (G) each decreased. Yarn thickness (T) remained relatively unchanged.

For Sample A, under a coursewise strain of 13%, yarn unit width (W) increased about 5%, yarn unit height (H) decreased about 14%, and yarn unit gap (G) decreased about 11%, from comparative dimensions in the un-deformed state. Under a coursewise strain of 20% (**78**), yarn unit width (W) increased about 13%, yarn unit height (H) decreased about 15%, and yarn unit gap (G) decreased about 12%, from comparative dimensions in the un-deformed state. The photograph in FIG. 17 shows Sample A under a 20% strain **78** in the course direction **80**. As strain increased in the coursewise direction **80**, yarn loops **22, 24** spread apart, causing less yarn contact. Thus, under loading in the coursewise direction **80**, an increasing yarn unit width (W), and a decreasing yarn unit height (H) and yarn unit gap (G) correlate with decreasing yarn contact.

For Sample B, under a coursewise strain of 12.5% (**82**), yarn unit width (W) increased about 11%, yarn unit height (H) had substantially no change, and yarn unit gap (G) decreased about 3%, from comparative dimensions in the un-deformed state. The photograph in FIG. 18 shows

Sample B under a 12.5% strain **82** in the course direction. Sample B has substantial yarn contact within a stitch even before deformation, or loading. As a result, as with loading in the walewise direction **74**, the variation in geometric parameters for Sample B during loading in the coursewise direction **80** is not as significant as for Sample A.

That is, under load in the course (horizontal) direction **80**, an increase in yarn unit width (W) results in a decrease in optical porosity and an increase in MER (increased contact resistance). Accordingly, optical porosity can be used as an index of sensitivity to compressive or tensile force under load in the course (horizontal) direction **80** in an embodiment of a method for controlling contact resistance in a textile-sensor.

## Experiment E

Thirty-three (**33**) sample fabrics each having a different stitch percentage of single jersey stitches **10**, miss stitches **34**, and tuck stitches **36**, were tested to determine variations in resistance relative to pressure in different stitch directions **74, 80**. The sample fabrics were then tested to determine variations in resistance relative to temperature in different stitch directions **74, 80**.

**Compression testing:** Each sample stitch pattern was tested for the effects of pressure, or loading, in both the course (horizontal) direction **80** and in the wale (vertical) direction **74**.

Under horizontal loading, resistance did not change significantly in most stitch patterns. As described herein, contact resistance varies according to the number, size, and shape of contact points in a particular direction **74, 80** of a textile structure. Thus, when there are fewer contact points in the course (horizontal) direction **80**, less change in resistance is expected in the horizontal direction **80**. For example, a high number of miss stitches **36** (such as the sample stitch pattern having 50% single jersey **10**, 35% miss **34**, and 15% tuck **36** stitches) results in fewer contact points in the course direction **80**. As a result, embodiments of a method for optimizing contact resistance in an electrically conductive yarn and textile can comprise selecting a yarn type and stitch pattern having fewer contact points in a course to provide a horizontal, low measurement sensitivity textile-sensor. Such a textile-sensor can be useful for measuring large compressive loads, such as across the ball of the foot in a sock designed for use in patients with diabetes.

Under vertical loading, resistance did change in many stitch patterns. In particular, testing showed that contact resistance can decrease with increased loading in the wale (vertical) direction **74**. Results of testing demonstrated that control of contact resistance relative to pressure is a function of the percentage of stitch type, which influences the number and quality of yarn contact points. For example, one sample stitch pattern having 50% single jersey **10**, 40% tuck **36**, and 10% miss **34** stitches, a higher percentage of tuck stitches **36** (and thus yarn contact points) than other samples, showed a strong linear relationship between increasing vertical loading and decreasing resistance. As a result, embodiments of a method for optimizing contact resistance in an electrically conductive yarn and textile can comprise selecting a yarn type and stitch pattern having a higher percentage of tuck stitches **36** (and thus yarn contact points) to provide a vertical, high measurement sensitivity textile-sensor. Such a textile-sensor can be useful for measuring vertically-oriented loads such as grip strength and duration or movement of an elbow in a patient undergoing rehabilitation.

It was discovered that under similar loads, resistance values were an order of magnitude higher in the vertical direction **74** than in the horizontal direction **80**. This variation is due in large part to the influence of tuck stitches **36**, particularly in the vertical direction **74**. As described herein with reference to FIGS. 3A and 3B, tuck stitch contact points **44**, tuck loop contact points **46**, held loop contact points **48**, and tensioned tuck stitch contact points **50** create increased yarn contact area (**52**), and thus provide control over contact resistance in a textile structure. In some embodiments of a method for controlling contact resistance in accordance with the present invention, placement of tuck stitches **36** can be utilized to optimize contact resistance in an electrically conductive textile-sensor in the vertical direction **74** along a wale. In other embodiments, tuck stitches **36** can be placed in multiple wales in a selected area of the fabric so as to optimize contact resistance in a defined area of the textile-sensor. In still other embodiments, selecting a stitch pattern having a particular high percentage of tuck stitches **36** that exhibits decreasing resistance with increasing load in both directions **74, 80**, such as the sample stitch pattern having 50% single jersey **10**, 40% tuck **36**, and 10% miss **34** stitches, contact resistance can be optimized in a textile-sensor in both directions **74, 80**. For example, such a stitch pattern can be knit in a defined area in a textile-sensor fabric to create a bi-directional sensing area for a particular use.

Temperature testing: Each of the 33 sample stitch patterns was tested for the effects of temperature on resistance in both the course (horizontal) direction **80** and in the wale (vertical) direction **74**. Findings showed that resistance (and thus electrical conductivity) varies in response to changing temperature for different stitch percentages and in different stitch directions **74, 80**.

In particular, findings showed that the relationship between temperature and resistance is linear. The samples having the largest percentage of tuck stitches **36** (which have the largest yarn contact area (**52**)) showed the best relationship (that is, the best  $R^2$  fit) between temperature and resistance. Results of testing demonstrated that control of contact resistance relative to temperature is a function of the percentage of stitch type, which influences the number and quality of yarn contact points (**42, 44, 46, 48, 50**). For example, one sample stitch pattern having 50% single jersey **10**, 40% tuck **36**, and 10% miss **34** stitches, a higher percentage of tuck stitches **36** (and thus yarn contact points) than other samples, showed a strong linear relationship between temperature and resistance.

As a result, embodiments of a method for optimizing contact resistance in an electrically conductive yarn and textile can comprise selecting a yarn type and stitch pattern having a larger percentage of tuck stitches **36** to provide a temperature-sensitive textile-sensor. Such a textile-sensor can be utilized for measuring ambient temperature in a heat-sensitive industrial environment, such as in a petrochemical production environment. Another embodiment of such a textile-sensor can be utilized for measuring a worker's skin temperature in an industrial setting, such as in a steel mill.

In some embodiments, contact resistance in electrically conductive yarns can be optimized in weft-knitted textile structures. In a weft-knitted fabric, one continuous yarn runs widthwise across the fabric and forms all of the loops **22, 24** in each course. Weft knit fabrics can be produced on both flat and circular knitting machines. In other embodiments, contact resistance in electrically conductive yarns can be optimized in warp-knitted textile structures. In a warp-knitted

fabric, one or more yarns generally run lengthwise in a zigzag pattern, which forms interlacing loops **22, 24** in two or more wales.

An electrically conductive textile having optimized contact resistance in accordance with the present invention can sense, or detect, a variety of variables in a person or object on which the textile is placed. For example, such a textile may sense physiological changes in a person wearing the textile. The detected change in a variable can be transmitted for monitoring, recording, and/or feedback. The sensed data may be in the form of an electrical signal. The signal transmission may be from the textile-sensor to a device on the textile and/or to another location. Such transmission or other operation related to the sensed data may be carried out via an electronic interface with the textile-sensor.

Embodiments of the present invention can include such an electronic interface with the textile-sensor. The electronic interface can include one or more of electronic circuitry configured to receive power from a power source, electronic circuitry configured for data transmission, an electronic device disposed on, mechanically affixed to, or integrated with the textile-sensor, a wired and/or wireless coupling between the textile-sensor and a portable electronic device, and/or other configurations to cooperate with any of a variety of different wearable or remote electronics. Such electronic interface is designed to avoid compromising the comfort and/or durability of a garment comprising the textile-sensor.

In one aspect of the present invention, the textile itself, having contact resistance optimized, acts as a sensor. Some embodiments of such a textile-sensor can measure variables or parameters such as tensile force, compressive force, movement, and temperature. Accordingly, various embodiments of such a textile-sensor can have different specific functionalities and applications. Embodiments of such a textile-sensor can include functionalities and applications related to, for example, (1) medical compression garments, (2) athletic compression garments, (3) hospital bed and/or wheelchairs, (4) fit of face masks, (5) cardiac monitoring; (6) EMG monitoring; (7) sensing temperature; (8) prosthetic limb enhancement; (9) sensing movement; (10) sensing force; and (11) intelligent bandages.

Some embodiments of a textile-sensor having optimized contact resistance can have applications in medical compression garments. In one embodiment, the textile-sensor can comprise a compressive pressure garment, such as a sock, that can be placed over a wound dressing. Using a resistive sensor configuration in the textile-sensor to measure compressive force, the compression sock can determine the average pressure applied across the sensor and transmit that information to a display device.

The ability to unobtrusively monitor the compressive pressure applied by such a sock to each patient allows for more consistent application of the desired level of compression to individual patients. Individualized compressive pressure therapy can lead to improved wound recovery, shorter healing time with reduced costs, and reduced risk of damage to the leg/limb from excessive compression. Such an embodiment overcomes a major limitation in conventional compression bandage product design—that is, that the compression level applied by a compression sock varies depending on the limb size of the patient (governed by physical laws such as Laplace's equation). For example, if the same product were used by ten different patients, each would experience a different actual applied compression level due to individual limb size variations.

In some embodiments, the textile-as-sensor can be integrated into compression hosiery to monitor product lifecycle and alert the user when a new compression product is indicated or desired. In addition, the textile-as-sensor can provide for continuous monitoring of compressive force during the period of medical necessity.

Some embodiments of a textile-sensor having optimized contact resistance can have applications in athletic compression garments. In some embodiments, the textile-sensor can be integrated into athletic compression garments to allow customer visualization of the desired correct compression at point-of-purchase. In addition, such a textile-sensor athletic compression garment can allow monitoring of the product lifecycle and alert the user when a new compression product is desired.

Some athletic garment embodiments comprise a vest capable of measuring physiological parameters for training. The vest can be capable of transmitting biological data to a smart phone, watch, or other visual display. Such a vest can monitor physiological metrics, including, for example, respiration rate, respiration volume, heart rate, and/or oxygen saturation.

Some embodiments of a textile-sensor having optimized contact resistance can have applications in hospital beds and/or wheelchairs. In some embodiments, the textile-sensor can be integrated into a hospital bed and/or wheelchair fabric in which the fabric surface is able to monitor temperature and/or compression. A layer of fabric with customised sensor size and shape can enable a patient or health care provider to detect when the patient is at risk of developing pressure ulcers from points of excessive pressure.

Some embodiments of a textile-sensor having optimized contact resistance can have applications in fitting of face masks. In some embodiments, the textile-sensor can be integrated into medical devices worn by patients both in a clinical and in an "at home" environment. For example, a textile-sensor medical device can comprise a face mask. The face mask textile-sensor can utilize compressive and tensile force measurements to establish proper fit, ensure comfort, and eliminate application of excessive force by the mask which may cause skin lesions. Such face mask textile-sensors can be worn, for example, by health care workers, by first responders, or by those as part of an industrial safety regime.

Some embodiments of a textile-sensor having optimized contact resistance can have applications in cardiac monitoring. Some embodiments of the present invention can comprise an electrically conductive yarn having contact resistance optimized for monitoring cardiac electrical signals. The cardiac sensing yarn can comprise a set, or plurality of sensors, positionable in various locations on a person for optimal sensing of cardiac signals. The cardiac sensing yarn having optimized contact resistance can comprise a stand-alone cardiac monitoring pad, or it can be integrally knit into desired locations in a textile-sensor. In the textile-sensor embodiment, each of the separate sensors can be connected to the other sensors with "wiring" pathways integrated into the textile structure. The cardiac monitor sensors can be connected to an electrocardiographic (ECG) output. Embodiments of the cardiac monitor textile structure can register electrical signals on the skin of both human and animal subjects, and can measure, record, and transmit cardiac waveform. Such a device can be utilized to monitor heart rate and/or ECG, for example, of athletes during activity, or perform ECG monitoring in clinical applications. Accordingly, embodiments of the cardiac monitor textile structure can provide an ambulatory sensing platform for

cardiac signals, including monitoring heart rate and/or ECG in medical and/or athletic applications.

Some embodiments of a textile-sensor having optimized contact resistance can have applications in electromyographic monitoring. Electromyography (EMG) is a technique used to record the electrical activity of skeletal muscles. This technique can use intra-muscular or skin surface electrodes to gather data. EMG as a technique can be used in medical illness, sports injury rehabilitation, as well as assisting in prosthetic integration and robot/human interfaces. In the medical sector, a primary use of EMG is in post stroke rehabilitation. EMG is used as a diagnostic tool to determine muscle strength. However, it may also be used to retrain and re-strengthen targeted muscles and associated neurons. This relatively new field requires physiological data in order to program game scenarios that allow the users to strengthen and retrain damaged muscles and neural pathways.

Some embodiments of a textile structure/sensor having optimized contact resistance according to the present invention may be utilized for electromyographic (EMG) monitoring. For example, such a textile structure may be worn to provide sensory feedback as part of neuromuscular rehabilitation.

Some embodiments of a textile-sensor having optimized contact resistance can have applications in sensing temperature. Some embodiments of a textile-sensor having optimized contact resistance may provide real-time monitoring of human temperature. The placement of such a textile-sensor within an armpit area of a baselayer garment allows real-time monitoring of body temperature and comparison with acceptable clinical parameters. In addition, placement of the textile structure on the exterior of a garment can provide real-time readings of environmental temperatures, which can be compared with health parameters and/or duty of care/safety requirements.

Experiment F illustrates that electrical resistance is dependent upon temperature. Thus, conductivity changes with temperature. Accordingly, an embodiment of a textile structure utilized for monitoring temperature can take expected temperature ranges into account when contact resistance in the textile structure is optimized.

In Experiment F, two uncoated fabric samples of single jersey stitch polyester and single jersey stitch merino wool were coated with polypyrrole (PPy) by vapour phase polymerization. 50 mm×50 mm samples of each fabric were placed in an aqueous solution of Iron (III) chloride (0.8 mol/L) and 1,5-naphthalenedisulfonic acid (0.1 mol/L) for one hour. The samples were removed and air dried. The dried samples were then suspended in a sealed vessel with pyrrole monomer at the bottom and heated to 60° C. for 3 hours. The samples were then removed, washed by warm water, and left to dry overnight.

Electrical resistivities of the samples were measured at temperatures at five-degree increments between 10° C. and 40° C. under argon by a multimeter connected to two copper strips on the fabric 30 mm apart. These results are shown in FIGS. 19 and 20. FIG. 19 is a table showing the measured resistivities for each of the polyester and the merino wool samples at each of the seven tested temperatures. FIG. 20 is a graph showing the resistivity measurements for each fabric sample plotted against the temperatures. For both fabric samples, there was a linear, inversely proportional relationship between temperature and resistivity. As temperature increased, resistivity decreased. The merino wool sample had

resistivity approximately half that of the polyester sample, due to the thicker nature of the wool fabric resulting in a better coating of polypyrrole.

Some embodiments of a textile-sensor having optimized contact resistance can have applications in prosthetic limb enhancement. People with prosthetic limbs lose the ability to "feel" objects. Nerves have been severed and therefore touch is lost. Neural engineering involves clinical implementation of devices in neural prosthesis systems for individuals with diseased or compromised neural systems so that pressures in such a system are transferred to nerve nodes within the surviving part of the limb. An example of such a pressure—nerve node interface is known as "neuromimetic interfaces" between neural tissue and engineered devices. A neuromimetic interface is defined as an electrode, polymer, or other device or material that mimics the mechanical, chemical, and/or electrical properties of neural tissue. An objective of neural engineering is to integrate such devices that behave as though they were natural neural tissue.

Some embodiments of a textile structure having optimized contact resistance according to the present invention can convert such pressures in an affected limb into an electrical signal and transfer those signals to nerve nodes within the surviving part of the limb. In other embodiments, peripheral nerve electrodes can combine electrical and optical stimulation techniques to effect a neuromimetic interface. In still other embodiments, polymeric fiber substrates with mechanical properties similar to neural tissue can be used in, or as, cortical electrodes.

Some embodiments of a textile-sensor having optimized contact resistance can have applications in monitoring movement. Some embodiments of a textile structure having optimized contact resistance according to the present invention can measure movement in a textile by a change in electrical resistance. Sensor placement and shape help determine what movement is measured and how it is measured. In some embodiments, a contact resistance-optimized textile-sensor can provide an average movement, rather than absolute movement. In certain embodiments, the textile-sensor can be combined with another sensor, for example, a conventional capacitance-type sensor. In such a combination, absolute movement can be measured with a high degree of sensitivity.

Examples of types of movement that can be monitored by some embodiments of a contact resistance-optimized textile structure (alone or in combination with another type of sensor) include: (1) simple respiration rate, in medical and/or athletic applications; (2) respiratory tidal volume, in medical and/or athletic applications; (3) limb movement, for example, in medical rehabilitation; (4) limb movement and joint angle, for example, in medical and sports rehabilitation; (5) robotic/human interface, for example, in medical, industrial, and at-risk first responders/military applications; and (6) subsurface monitoring, for example, monitoring structural and/or earthquake-type movement, and monitoring in geotechnical real-time and related to disaster prevention applications.

Some embodiments of a textile-sensor having optimized contact resistance can have applications in monitoring force. Some embodiments of a textile structure having optimized contact resistance according to the present invention can measure both tensile and compressive force by a change in electrical resistance. Such an embodiment can measure absolute compressive force and/or average tensile force. Such an embodiment can be utilized to monitor these forces in applications, including: (1) pressure sensors, in medical and/or athletic applications; (2) compressive medical ban-

dages; (3) limb strength/power, for example, in advanced medical and sports rehabilitation; (4) ambulatory blood pressure monitoring; and (5) subsurface monitoring, for example, in structural and "disaster" forces, geotechnical real-time, and disaster prevention applications.

Some embodiments of a textile-sensor having optimized contact resistance can have applications in intelligent bandages. Some such embodiments of a textile structure can be utilized in production of "intelligent" bandages. Such bandages may sense temperature, force, moisture, and/or pH. In certain embodiments, the contact resistance-optimized textile-sensor can sense microcirculation of limb extremities.

Embodiments of a method for optimizing contact resistance in electrically conductive yarns and textiles, and textiles having such optimized contact resistance, of the present invention can comprise selecting a sensing activity for the textile; selecting a combination of variables from the group consisting of yarn variables, stitch variables, and textile variables; and knitting an electrically conductive yarn in the textile in accordance with the selected combination of variables, wherein the knitted combination of variables provides an optimal contact resistance in the textile correlated with a desired electrical conductivity for the sensing activity. In some embodiments, the knitted combination of variables provides a predictable yarn contact area (52) for the electrically conductive yarn correlated with the optimal contact resistance. In some embodiments, the yarn contact area (52) comprises a size and a shape, and the knitted combination of variables provides a predictable number and quality of yarn contact points (42, 44, 46, 48, 50) associated with the size and shape of the yarn contact area (52).

The combination of variables can be selected from yarn variables, including yarn type, yarn fabrication method, and yarn count. The combination of variables can be selected from stitch variables including stitch pattern, stitch length, and stitch percentage. The combination of variables can be selected from textile variables including electrical resistivity, fabric thickness, fabric weight, optical porosity, and percentage permanent stretch. In some embodiments, the stitch variables including stitch pattern can be selected from miss stitches 34, tuck stitches 36, and jersey stitches 10. Some embodiments can further include selecting a measurement sensitivity for the sensing activity, and the knitted combination of variables can provide the optimal contact resistance in the textile correlated with a desired electrical conductivity for the measurement sensitivity. In certain embodiments, selecting a sensing activity for the textile can further include selecting a plurality of different sensing activities for the textile. In various embodiments, the sensing activity can be selected from sensing tensile force, compressive force, movement, temperature, and physiological activity.

Other embodiments of a method for optimizing contact resistance in electrically conductive yarns and textiles, and textiles having such optimized contact resistance, can comprise selecting a combination of variables from the group consisting of yarn variables, stitch variables, and textile variables; and knitting an electrically conductive yarn having a yarn contact area in the textile in accordance with the selected combination of variables, wherein the knitted combination of variables provides a controllable amount of contact resistance in the textile. Some embodiments can further include selecting a sensing activity for the textile, and a controlled amount of contact resistance in the textile is correlated with a desired electrical conductivity for the sensing activity. In such an embodiment, the combination of variables can be selected from yarn variables including yarn

type, yarn fabrication method, and yarn count. The combination of variables can be selected from stitch variables including stitch pattern, stitch length, and stitch percentage. The combination of variables can be selected from textile variables including electrical resistivity, fabric thickness, fabric weight, optical porosity, and percentage permanent stretch. In some embodiments, the stitch variables including stitch pattern can be selected from miss stitches 34, tuck stitches 36, and jersey stitches 10.

Some embodiments can further include increasing the size of the yarn contact area (52) to decrease the contact resistance. The yarn contact area (52) comprises a number and size of yarn contact points (42, 44, 46, 48, 50). Some embodiments can further include selecting an increased stitch length 20 to increase the number and size of yarn contact points (42, 44, 46, 48, 50) and the size of the yarn contact area (52), thereby decreasing the amount of contact resistance. Other embodiments can further include selecting stitch percentage of the miss stitches 34, tuck stitches 36, and jersey stitches 10 to control the number and size of yarn contact points (42, 44, 46, 48, 50) and the size of the yarn contact area (52), and thereby control the amount of contact resistance. Still other embodiments can further include selecting yarn type from the group consisting of filament yarn and staple fiber yarn to control the number and size of yarn contact points (42, 44, 46, 48, 50) and the size of the yarn contact area (52), and thereby control the amount of contact resistance. In such embodiments, yarn type can be selected from natural yarn and synthetic yarn. Still other embodiments can further include selecting an increased yarn count to increase the number and size of yarn contact points (42, 44, 46, 48, 50) and the size of the yarn contact area (52), thereby decreasing the amount of contact resistance.

Some embodiments can further include selecting an increased fabric thickness to increase the size of the yarn contact area (52), thereby decreasing the amount of contact resistance. Some embodiments can further include selecting an increased stitch percentage of miss stitches 34 and tuck stitches 36. Other embodiments can further include selecting an increased fabric weight to increase the size of the yarn contact area (52), thereby decreasing the amount of contact resistance. In such an embodiment, selecting an increased fabric weight can further include selecting an increased stitch percentage of miss stitches 34 and tuck stitches 36. Other embodiments can further include selecting a decreased optical porosity to increase the size of the yarn contact area (52), thereby decreasing the amount of contact resistance. In such an embodiment, selecting a decreased optical porosity can further include selecting an increased stitch percentage of tuck stitches 36. Still other embodiments can further include selecting a decreased percentage permanent stretch to increase the size of the yarn contact area (52), thereby decreasing the amount of contact resistance.

In some embodiments, the electrically conductive yarn in the textile can further include a resting mean electrical resistivity (MER) in the textile, and stitch percentage of the miss stitches 34, tuck stitches 36, and jersey stitches 10 can be selected to decrease the resting MER and the amount of contact resistance.

Some embodiments can further include selecting a measurement sensitivity for the sensing activity, and a controlled amount of contact resistance in the textile can be correlated with a desired electrical conductivity for the measurement sensitivity. In some embodiments, a measurement sensitivity can be selected from the group consisting of tensile force, compressive force, movement, temperature, and physiologi-

cal activity. In some embodiments, the electrically conductive yarn in the textile can further include a mean electrical resistivity (MER), and stitch percentage of the miss stitches 34, tuck stitches 36, and jersey stitches 10 can be selected to provide a particular dynamic range in MER to control the measurement sensitivity during deformation of the textile. In particular, the dynamic range in MER can comprise a large dynamic range in MER to optimize the contact resistance for decreased measurement sensitivity for reliable measurements of compressive force over a large force range. Alternatively, the dynamic range in MER can comprise a small dynamic range in MER to optimize the contact resistance for increased measurement sensitivity for reliable measurements of compressive force over a small force range.

In some embodiments, the electrically conductive yarn in the textile can further include a mean electrical resistivity (MER), and stitch percentage of the miss stitches 34, tuck stitches 36, and jersey stitches 10 can be selected to provide a narrow range of MER variation to optimize the contact resistance for increased measurement sensitivity for reliable measurements of light weight pressures. In other embodiments, the electrically conductive yarn in the textile can further include an optical porosity, and a particular optical porosity can be selected to optimize the contact resistance to control the measurement sensitivity for compressive or tensile force loads. In particular, the optical porosity can comprise a low optical porosity to decrease the contact resistance for increased measurement sensitivity. Alternatively, the optical porosity can comprise a high optical porosity to increase the contact resistance for decreased measurement sensitivity. In some embodiments, stitch percentage of the miss stitches 34, tuck stitches 36, and jersey stitches 10 can be selected to optimize the amount of contact resistance to control temperature measurement sensitivity.

In certain embodiments of such a method, selecting a sensing activity for the textile can further include selecting a plurality of different sensing activities for the textile. In various such embodiments, the sensing activity can be selected from sensing tensile force, compressive force, movement, temperature, and physiological activity.

Some embodiments of a textile according to the present invention can comprise a sensing area comprising an electrically conductive yarn knitted in the textile and adapted for a sensing activity; and the sensing area comprising a combination of variables selected from the group consisting of yarn variables, stitch variables, and textile variables, wherein the combination of variables provides an optimal contact resistance in the textile correlated with a desired electrical conductivity for the sensing activity. In some embodiments, the combination of variables can comprise a predictable yarn contact area (52) for the electrically conductive yarn correlated with the optimal contact resistance. In some embodiments, the yarn contact area (52) can further include a size and a shape, and the combination of variables can further include a predictable number and quality of yarn contact points (42, 44, 46, 48, 50) associated with the size and shape of the yarn contact area (52).

The combination of variables can be selected from the group consisting of yarn type, yarn fabrication method, and yarn count. In some embodiments of such a textile, the combination of variables can be selected from the group consisting of stitch pattern, stitch length, and stitch percentage. In some embodiments of such a textile, the combination of variables can be selected from the group consisting of electrical resistivity, fabric thickness, fabric weight, optical porosity, and percentage permanent stretch. The stitch vari-

29

ables comprising stitch pattern can be selected from the group consisting of miss stitches 34, tuck stitches 36, and jersey stitches 10.

In some embodiments of such a textile, the sensing activity can comprise a measurement sensitivity, and the combination of variables comprises the optimal contact resistance in the textile correlated with a desired electrical conductivity for the measurement sensitivity. Some embodiments of such a textile can further include a plurality of sensing areas, and each of the sensing areas can be adapted for a different sensing activity. In some embodiments of such a textile, the sensing activity can be selected from sensing tensile force, compressive force, movement, temperature, and physiological activity.

Some embodiments of a textile according to the present invention can comprise a sensing area comprising an electrically conductive yarn knitted in the textile; and the sensing area comprising a combination of variables selected from the group consisting of yarn variables, stitch variables, and textile variables, wherein the combination of variables provides a controllable amount of contact resistance in the textile. The sensing area can be adapted for a sensing activity, and a controlled amount of contact resistance in the textile can be correlated with a desired electrical conductivity for the sensing activity. In some embodiments, the combination of variables can be selected from the group consisting of yarn type, yarn fabrication method, and yarn count. In some embodiments, the combination of variables can be selected from the group consisting of stitch pattern, stitch length, and stitch percentage. In some embodiments, the combination of variables can be selected from the group consisting of electrical resistivity, fabric thickness, fabric weight, optical porosity, and percentage permanent stretch. The stitch variables comprising stitch pattern can be selected from the group consisting of miss stitches 34, tuck stitches 36, and jersey stitches 10.

In some embodiments of the textile, the sensing activity can comprise a measurement sensitivity, and the combination of variables can comprise the optimal contact resistance in the textile correlated with a desired electrical conductivity for the measurement sensitivity. Some embodiments of the textile can further include a plurality of sensing areas, and each of the sensing areas can be adapted for a different sensing activity. In some embodiments of such a textile, the sensing activity can be selected from sensing tensile force, compressive force, movement, temperature, and physiological activity.

A method for optimizing contact resistance in electrically conductive yarns and textiles and textiles having such optimized contact resistance according to the present invention provides advantages over conventional approaches to construct electrically conductive yarns and textiles. One advantage is that embodiments of the present invention comprise a method for designing a textile structure to optimize the position and size of yarn contact areas (52) that allows control of electrical contact resistance and thus sensitivity of the textile structure. Thus, such a method provides a basis for varying a textile structure for specific applications. As a result, such a method can be utilized in a wide variety of applications and products.

Another advantage is that embodiments of the present invention utilize predictable characteristics and variables of yarns and textiles that improve control of contact resistance. Accordingly, embodiments of the present invention provide for optimization of contact resistance in electrically conductive yarns in a simple, cost-effective, and repeatable manner.

30

Another advantage is that embodiments of the present invention allow use of a single electrically conductive fiber type in a textile sensor.

Another advantage is that embodiments of a "textile-sensor" of the present invention provide the capability integrated into a textile to monitor a plurality of point outputs (such as physiological variables), thus allowing a more comprehensive and/or averaged measurement of such outputs.

Another advantage is that embodiments of the present invention allow a textile structure having optimized contact resistance to be utilized as a sensor for force, pressure, movement, temperature, and/or physiological activity.

Another advantage is that embodiments of the present invention thus providing enhanced sensing capabilities of such fabrics can be incorporated into composite structures. Such combination sensors can provide either passive or active sensing platforms. In one application, such sensors can be utilized to remotely measure physiological output of the human body. A variety of data obtainable utilizing such fabrics can be used, for example, to improve health outcomes, to enhance safety among athletes, first responders, and soldiers, and for industrial applications.

Another advantage is that embodiments of the present invention comprising knitted fabrics can provide superior draping characteristics (ability to form on organic shapes) over woven materials, thereby enhancing user comfort, durability, and cost.

In addition, some embodiments of the present invention provide advantages in manufacturing over conventional textile-based sensors. For example, such a method can be implemented using computer aided design (CAD) programming prior to manufacture, thereby preventing wasted labor, machinery, and materials costs for trial and error construction. A CAD system programmed for manufacturing a textile structure having optimizing contact resistance can be used to create such a textile structure when the flexible conducting network of electrically conductive yarn is at rest or when subjected to tension or compression. Stitch and yarn variables controllable for optimizing contact resistance in a textile structure can be implemented with CAD software usable in existing commercial knitting machines. Thus, embodiments of the present invention can provide the advantages of simplified design and manufacturing processes with significant reductions in costs as compared to existing textile sensors. By using existing commercial equipment, embodiments of the present invention can further provide the advantage of a means for repeatably producing a durable resistive textile-sensor.

Although the present invention has been described with reference to particular embodiments, it should be recognized that these embodiments are merely illustrative of the principles of the present invention. Those of ordinary skill in the art will appreciate that a method for optimizing contact resistance in electrically conductive yarns and textiles and yarns and textiles so optimized of the present invention may be constructed and implemented in other ways and embodiments. Accordingly, the description herein should not be read as limiting the present invention, as other embodiments also fall within the scope of the present invention.

What is claimed is:

1. A textile having at least one fully integrated knitted sensor, the textile; comprising:  
at least one sensing area adapted for a sensing activity,  
wherein the sensing activity is selected from the group consisting of: tensile force, compressive force, movement, temperature and physiological activity, and

**31**

wherein the at least one sensing area comprises an electrically conductive yarn knitted in the textile; the at least one sensing area comprising a combination of stitches selected from two or more of the group consisting of: jersey stitches, miss stitches, and tuck stitches; wherein the combination of stitches in the at least one sensing area provides a controllable amount of contact resistance in the textile, and wherein the controllable amount of contact resistance in the textile is correlated with a desired electrical conductivity for the sensing activity.

2. The textile of claim 1, wherein the textile further comprises an electrical resistivity, fabric thickness, fabric weight, an optical porosity, and percentage permanent stretch, which provide a controllable amount of contact resistance in the textile.

3. The textile of claim 1, wherein the sensing activity comprises a measurement sensitivity, and wherein the at least one sensing area comprises the controlled contact resistance in the textile correlated with a desired electrical conductivity for the measurement sensitivity.

4. The textile of claim 1, further comprising a plurality of the at least one sensing areas, wherein each of the sensing areas is adapted for a different sensing activity.

5. The textile of claim 1, wherein at least 50% of the stitches in the combination of stitches in the at least one sensing area comprise jersey stitches, and wherein the remaining 50% of stitches comprises a combination of miss stitches and tuck stitches.

**32**

6. The textile of claim 1, wherein a percentage of miss stitches in the combination of stitches comprised in the at least one sensing area is at least 5% and at most 45%.

7. The textile of claim 1, wherein a percentage of tuck stitches in the combination of stitches comprised in the at least one sensing area is at least 5% and at most 45%.

8. The textile of claim 1, wherein the electrically conductive yarn is defined by a yarn type, a yarn fabrication method, and a yarn count, and wherein the combination of yarn type, yarn fabrication method, and/or yarn count provides further control over the amount of contact resistance in the textile.

9. The textile of claim 1, wherein the electrically conductive yarn in the textile further comprises a mean electrical resistivity (MER), wherein the sensing activity comprises sensing compressive force, and wherein the dynamic range in MER controls the measurement sensitivity during deformation of the textile.

10. The textile of claim 1, wherein the sensing activity comprises sensing physiological activity, and wherein physiological activity comprises an activity selected from one or more of the group consisting of: cardiac monitoring; muscle activity monitoring; and brain wave signal sensing.

11. A garment comprising the textile of claim 1.

12. The garment of claim 11, wherein the garment comprises a medical garment and wherein the sensing activity of the textile comprises sensing average compressive force applied by the garment.

13. The garment of claim 11, wherein the garment comprises an athletic garment capable of monitoring physiological metrics.

\* \* \* \* \*